



US007732059B2

(12) **United States Patent**  
Ren et al.

(10) **Patent No.:** US 7,732,059 B2  
(45) **Date of Patent:** Jun. 8, 2010

(54) **HEAT EXCHANGER TUBING BY  
CONTINUOUS EXTRUSION**

(75) Inventors: **Baolute Ren**, Lititz, PA (US); **Raymond J. Kilmer**, Lancaster, PA (US); **John F. Butler, Jr.**, Lititz, PA (US)

(73) Assignee: **Alcoa Inc.**, Pittsburgh, PA (US)

(\*) Notice: Subject to any disclaimer, the term of this patent is extended or adjusted under 35 U.S.C. 154(b) by 1298 days.

(21) Appl. No.: **11/157,668**

(22) Filed: **Jun. 21, 2005**

(65) **Prior Publication Data**

US 2006/0118282 A1 Jun. 8, 2006

**Related U.S. Application Data**

(60) Provisional application No. 60/633,076, filed on Dec. 3, 2004.

(51) **Int. Cl.**  
**B32B 15/20** (2006.01)  
**B32B 15/02** (2006.01)

(52) **U.S. Cl.** ..... **428/654**; 148/439; 420/528;  
165/905

(58) **Field of Classification Search** ..... None  
See application file for complete search history.

(56) **References Cited**

## U.S. PATENT DOCUMENTS

- 3,765,216 A 10/1973 Green  
4,238,248 A \* 12/1980 Gyongyos et al. ..... 148/551  
5,000,025 A 3/1991 Beekel ..... 72/259  
5,015,439 A 5/1991 Tyler et al. ..... 419/23  
5,353,639 A 10/1994 Brookins et al. ..... 72/363  
5,514,228 A \* 5/1996 Wyatt-Mair et al. ..... 148/551  
5,634,991 A \* 6/1997 Kamat ..... 148/551  
5,976,278 A \* 11/1999 Sircar ..... 148/550  
6,059,902 A \* 5/2000 Yoshihara et al. ..... 148/550

- 6,391,127 B1 \* 5/2002 Wyatt-Mair et al. ..... 148/551  
6,458,224 B1 \* 10/2002 Ren et al. ..... 148/437  
6,500,284 B1 \* 12/2002 Zhou et al. ..... 148/551  
6,503,446 B1 1/2003 Ren et al.  
6,536,255 B2 3/2003 Kraft ..... 72/256  
6,602,363 B2 8/2003 Ren  
6,656,296 B2 12/2003 Ren et al.  
6,660,107 B2 12/2003 Ren  
6,739,387 B1 5/2004 Ren ..... 165/176  
2004/0086417 A1 \* 5/2004 Baumann et al. ..... 420/531

(Continued)

## FOREIGN PATENT DOCUMENTS

DE 3810261 A1 3/1988

(Continued)

## OTHER PUBLICATIONS

Journal—Rudy I Metale Niezelazne(Enclosed), Nov. 1998.

(Continued)

Primary Examiner—John J Zimmerman

(74) Attorney, Agent, or Firm—Greenberg Traurig, LLP

(57) **ABSTRACT**

A heat exchanger tube having enhanced corrosion resistance and improved resistance to high burst pressures. The heat exchanger tube comprises an aluminum alloy that consists essentially of about 0.01-1.5% silicon, up to about 1.2% copper, up to about 2.0% manganese, about 0.01-1.0% iron, about 0.01-5.0% zinc, up to about 0.02% titanium and the balance substantially aluminum and incidental elements and impurities.

**23 Claims, 3 Drawing Sheets**

U.S. PATENT DOCUMENTS

2005/0126745 A1\* 6/2005 Bowles et al. .... 164/490  
2006/0088438 A1\* 4/2006 Corrigan et al. .... 420/532  
2006/0196635 A1\* 9/2006 Lesage .... 165/76

FOREIGN PATENT DOCUMENTS

JP 59-143039 \* 8/1984  
JP 2002-294383 \* 10/2002  
WO WO 9117002 3/1991 .... 516/749

OTHER PUBLICATIONS

Journal—Light Metal Age (Enclosed), Aug. 1995.

Journal—Extrusion Goes Continuous; process Promises Economies (Enclosed), Dec. 1984.

Journal—CME Chartered Mechanical Engineer (Enclosed), Feb. 1984.

Article—Tube Manufacture by the 'Conform' Process, Sep. 1982.

Conference Paper—5th International Aluminum Extrusion Technology Seminar, vol. II (Table of Contents), including "New Developments in Conform Technology for Continuous Extrusion", pp. 413-419, and "The Development of Microstructure and the Consolidation of RSP Aluminum Alloys in Conform Extrusion", pp. 427-438, 1977.

Journal—Fils Bandes Profiles, Paris, Apr. 21-22, 1977.

A Review of the Confex Continuous Non Ferrous Extrusion Process, by David Godwin, Confex Technology, Ltd., pp. 571-577, 1998.

\* cited by examiner



FIG. 1



FIG. 2

CONTINUOUSLY CASTING A FEEDSTOCK ROD

EXTRUDING THE FEEDSTOCK ROD THROUGH A  
CONTINUOUS ROTARY EXTRUSION PROCESS TO FORM  
A MICRO MULTI VOID TUBE

QUENCHING THE MICRO MULTI VOID TUBE

FIG. 3



FIG. 4



FIG. 5



FIG. 6



FIG. 7A



FIG. 7B



FIG. 8

## 1

HEAT EXCHANGER TUBING BY  
CONTINUOUS EXTRUSIONCROSS REFERENCE TO RELATED  
APPLICATIONS

This application claims the benefit of U.S. Provisional Application Ser. No. 60/633,076, filed on Dec. 3, 2004, the disclosure of which is fully incorporated by reference herein.

## FIELD OF THE INVENTION

The present invention relates to a single and multiple layer aluminum tube and a method for economically fabricating such a tube. More specifically, this invention discloses a method for manufacturing aluminum tube products with thin walls and fine features, such as micro multi void tubing, used in the manufacture of heat exchangers.

## BACKGROUND OF THE INVENTION

Aluminum heat exchangers are used widely in the automotive industry. Applications include engine cooling systems where heat exchangers such as radiators, oil coolers, charge air coolers and the like are employed. Additionally, passenger climate control systems also utilize heat exchangers as evaporators and condensers. Air conditioning systems typically have two heat exchangers: condensers and evaporators. Condensers typically operate at elevated pressures (>500 psi) and most typically are made with extruded tubes. These tubes are produced via traditional methods of extrusion. Most radiators use tubes made from welded or folded sheet (in part, due to the elevated costs per unit length of extruded tubes versus tubes made from sheet and in part as a result of the lower system pressure requirements of radiators (typically 20 psi or less)). However, some radiator tubes are also manufactured by extrusion processes depending on the design and specific durability requirements of the radiator in the field.

Typical extrusion based heat exchangers come essentially in two designs. The first design uses round tubing and bare (i.e. unclad) fins that are mechanically attached to the round tubes by first lacing the tubes into holes punched in the fins, and then expanding the tubes to ensure that the tube's outer surface is in close mechanical contact with the fins.

The second typical design uses flat tubing having a plurality of channels in the tubing, commonly referred to as multi void tubing or micro multi void tubing. This type of heat exchanger tubing is attached to the fins using a brazing process. The cross section of the flow channels can vary, e.g., circular, oval, square, rectangular, or other regular or irregular shapes. Typically, micro multi void and multi void tubing are about 10-60 mm in width and about 1-2 mm in height.

Most aluminum extruded tubing products made for heat exchanger systems are produced by using traditional billet extrusion methods, such as press extrusion. As the alloy strength increases, the ability to use these traditional methods of extrusion becomes less feasible due to the difficulty of extruding the high strength alloy into a small tube. This difficulty occurs because as the dimensions of the heat exchanger tube decreases, the extrusion ratio, which is defined by a ratio of container bore area and the total cross sectional area of extrusion, increases thereby increasing the extrusion pressure needed to extrude the heat exchanger tube. The end result is that it is difficult (or sometimes not possible) and at the least, very expensive to produce fine dimensioned tubing from high strength materials using traditional extrusion methods. This is becoming a barrier to the introduction

## 2

of newer heat exchanger designs that utilize fine dimensioned tubing, particularly for next generation designs where tubing must withstand very high pressures, for example CO<sub>2</sub> refrigerant systems. In addition, as the heat exchanger manufacturers continue to work on next generation designs there is an increasing need for thin walled tubing with finer features that has high strength and high corrosion resistance, and in some instance high strength at elevated service temperature. Therefore, heat exchanger tubing might soon be required to operate at significantly higher pressures while at the same time becoming smaller in size as compared to current heat exchanger designs with tubes that use R-134a as the refrigerant. In order to meet these increasing demands in a cost effective manner, it is critical that the heat exchanger tubes be extruded from higher strength alloys.

Therefore, there exists a need for an improved high strength heat exchanger tube that can withstand high burst pressures, exhibit good corrosion resistance, have small dimensions (e.g. 10 mm by 1 mm MMV tubing with micro void width less than 1 mm), and have fine internal features. Additionally, there exists a need for a process to economically fabricate such a tube.

A continuous rotary extrusion process, known as the Conform™ Process, was developed and patented (U.S. Pat. No. 3,765,216) by the United Kingdom Atomic Energy Authority. In the Conform™ Process a rod or particulate feedstock replaces the extrusion billet and thereby making the extrusion process continuous. The equipment used in the Conform™ Process includes a grooved wheel, a coining roll, an abutment, a close fitting shoe, and an extrusion die. During the extrusion process the feedstock is fed into a space formed by the grooved wheel, close fitting shoe, and abutment, and is heated and pressurized by the friction between the rotating wheel and metal. When the metal temperature is sufficiently high the pressure extrudes the metal through the extrusion die.

For high volume aluminum tubing production requiring high productivity (lbs/hr), capital investment generally has not particularly favored the Conform™ process (vs. the traditional billet extrusion process) because of developed multi-out capabilities of billet extruders (sometimes up to 8 out) and differences in market pricing for feedstock rod vs. billet (i.e. billet is generally cheaper per pound for a specific alloy). Furthermore, it is a general perception in the industry that the Conform™ process is more appropriate for simple, larger tolerance, less demanding shapes made from easy to extrude alloys like AA1060 for products such as spacer bars and the like. Hence the overwhelming majority of tubing is produced today via traditional billet based extrusion processes.

However, the Conform™ process can make certain shapes with certain metallurgical structures that billet based process cannot make due to the process differences between the two processes, namely due to the differences in metallurgical structure of the rodstock and the reduced extrusion ratios (and resulting constancy of the die face pressure) of the Conform™ process.

Thus, there is a problem in the art, associated with the difficulty in extruding a small tube having a relatively complex structure, such as a micro multi void tubing, from a material with a high flow stress because the small tubing size increases the extrusion ratio, i.e. the cross sectional area ratio between the billet and the extruded product. This in turn increases the tonnage of pressure needed to extrude the alloy into the desired shape and dimension, and effectively limits the alloy chemistries that can be chosen as well as the allowable base microstructure of the metal being extruded to microstructures that have low flow stresses. Hence billets are

generally homogenized prior to extrusion, solute contents are generally low, and the billets are generally DC cast and pre-heated immediately prior to extrusion process.

#### SUMMARY OF THE INVENTION

The present invention is a response to the need for an improved heat exchanger tube, providing a method for producing an improved aluminum or heat exchanger tube at reduced costs and reduced manufacturing times while utilizing higher strength alloys. The invention is further directed to a heat exchanger tube having improved resistance to high burst pressures.

The heat exchanger tube is comprised of an aluminum alloy that consists essentially of about 0.01-1.5% silicon, up to about 1.2% copper, up to about 2.0% manganese, about 0.01-1.0% iron, up to about 5.0% zinc, up to about 0.02% titanium, and the balance substantially aluminum and incidental elements and impurities. The aluminum alloy can further contain one or more of the following elements: about 0.01-0.35% chromium, about 0.01-0.35% zirconium, about 0.01-0.35% vanadium, about 0.01-0.35% cobalt, up to about 1.0% magnesium, and about 0.01-2.5% nickel. The aluminum alloy is a feedstock that can be fabricated using processes that are commonly known in the art.

In one embodiment, the feedstock can also be fabricated using a continuously cast process. The feedstock could be a strip, rod, or sheet having an aspect ratio ranging from about 1:1 to 500:1. The feedstock may also be exposed to elevated temperatures greater than about 300° C. The feedstock has an average secondary dendrite arm spacing of less than about 100 microns, has a cross sectional area of about 2500 mm<sup>2</sup> or less and has a yield strength ranging from about 50 to about 150 MPa. The feedstock is then extruded using a continuous rotary extrusion process.

After extrusion, the extrusion (e.g. heat exchanger tube) can be quenched using quenching processes that are commonly known in the art, such as still air cooling, forced air cooling, spray water cooling, immersion in water, spray coolant cooling or immersion in coolant.

In one embodiment, the heat exchanger tube can further comprise a zinc coating of at least about 80 wt % zinc that is located on the exterior surface of the tube. The zinc coating can be applied to the exterior surface by coating processes that are commonly known in the art such as thermal spray, chemical vapor deposition, physical vapor deposition, cold spray or other metal deposition systems.

In one embodiment, the heat exchanger tube has a circumference less than about 400 mm.

In one embodiment, the heat exchanger tube is a micro multi void tube with a maximum height not exceeding about 5 mm.

In one embodiment, one or more walls of the heat exchanger tube have a wall thickness of less than about 1 mm.

In one embodiment, the heat exchanger tube has a post brazed tensile yield strength that exceeds about 35 MPa, preferably said tube has a post brazed tensile yield strength that exceeds about 45 MPa.

In one embodiment, the heat exchanger tube can withstand a burst pressure greater than about 69 bar. Similarly, the post braze heat exchanger tube can also withstand a burst pressure greater than about 69 bar.

In one embodiment, the heat exchanger tube could have an electric conductivity that is above 48% IACS (International Annealed Copper Standard). The post braze heat exchanger tube could have an electric conductivity that is above 48% IACS.

In one embodiment, the invention is directed to a multi layered extruded tube having improved resistance to high burst pressures. The multi layered tube has an inner core tube comprising an aluminum alloy consisting essentially of about 0.01-1.5% silicon, up to about 1.2% copper, up to about 2.0% manganese, about 0.01-1.0% iron, up to about 5.0% zinc, up to about 0.02% titanium, and the balance substantially aluminum and incidental elements and impurities, and one or more clad layers comprising an aluminum alloy selected from 10 the group consisting essentially of the 1XXX, 2XXX, 3XXX, 4XXX, 5XXX, 6XXX, 7XXX, and 8XXX series of aluminum alloys cladded on an exterior surface of said inner core. The inner core tube can further contain one or more of the following elements: about 0.01-0.35% chromium, about 15 0.01-0.35% zirconium, about 0.01-0.35% vanadium, about 0.01-0.35% cobalt, up to about 1.0% magnesium and about 0.01-2.5% nickel.

In one embodiment, the aluminum alloy used for the inner core is a feedstock that can be fabricated using processes that 20 are commonly known in the art. The feedstock can also be fabricated using a continuously cast process. The feedstock could be a strip, rod, or sheet having an aspect ratio ranging from about 1:1 to 500:1. The feedstock may also be exposed to elevated temperatures greater than about 300° C. The feedstock has an average secondary dendrite arm spacing of less than about 100 microns, has a cross sectional area of about 2500 mm<sup>2</sup> or less and has a yield strength ranging from about 50 to about 150 MPa. The feedstock is then extruded using a continuous rotary extrusion process into an extrusion.

After extrusion, the extrusion (e.g. inner core tube) can be quenched using quenching process processes that are commonly known in the art such as still air cooling, forced air cooling, spray water cooling, immersion in water, spray coolant cooling or immersion in coolant.

One or more tangential continuous rotary extrusion machines is used to clad one or more clad layers onto the exterior surface of the inner core tube.

After cladding, one or more of the cladded layers can be drawn or sintered over the inner core tube.

40 The multi layered extruded tube can further comprise a zinc coating of at least about 80 wt % zinc that is located on the exterior surface of the tube. The zinc coating can be applied to the exterior surface by coating processes that are commonly known in the art such as thermal spray, chemical vapor deposition, physical vapor deposition, cold spray or other metal deposition systems.

One or more of the clad layers in the multi layered extruded tube can be selected from the Aluminum Association's 4343, 4045 and 4047 aluminum alloys, and have a thickness ranging from about 3 μm to about 300 μm.

One clad layer could have an electrochemical potential difference of at least about 20 mV to about 40 mV (positive or negative) when compared to the inner core tube or an adjacent clad layer as defined by the ASTM G69 standard.

55 The multi layered extruded tube can be a micro multi void heat exchanger tube having a circumference less than about 400 mm and a height not exceeding about 5 mm.

The feedstock is fabricated by using, but not limited to, continuous casting followed by warm and cold work into rod, bar, plate, sheet, and other shapes that are used for the Conform™ Process. (While it is possible to fabricate feedstock from DC (direct chill) based ingot process, it is generally more costly and the slower solidification rates are generally less advantageous). The continuous casting process is controlled such that the metallurgical structure is obtained to meet the physical, electrochemical, and mechanical property requirements for the extruded tube products. For instance, the

composition and solidification process can be controlled such that the alloy has high solute in solid solution, fine particles for dispersoids strengthening, and balanced electrochemical potentials between particles and matrix for excellent corrosion resistance. The stock is thermally treated or non-thermally treated according to the property requirements of the final product, which typically include mechanical properties, corrosion resistance, fatigue resistance, etc. For example, it is possible to form after braze, in the area where the extrusions come in contact with molten 4xxx braze cladding, a dispersoid band of  $\text{Al}_{12}(\text{Fe},\text{Mn})_3\text{Si}$  particles in a low (<0.1%) Si 3003 type alloy after brazing, if the stock is not homogenized prior to rotary extrusion. This post-brazed microstructure has been shown to be highly corrosion resistant in splash type environment in cars such as sheet based heat exchangers like radiators.

The continuous cast feedstock properties, such as dispersoid populations or solute contents in solid solution, can be nearly retained in the final product due to a short thermal cycle in the Conform™ Process. In the billet extrusion process, the billets are almost always homogenized and then heated up to extrusion temperature before extrusion. During the billet homogenization, cooling after homogenization and extrusion preheat processes some alloying elements in the billet precipitate. The solute precipitation changes the billet's metallurgical structure and the resultant properties of final products. The Conform™ process itself does not rely on a forced pre-heating step to elevate the material's temperature (and hence lower the flow stress) to extrude the material through the die(s). Immediately prior to Conform™ extrusion, the rod stock is fed into the wheel at room temperature and the material undergoes tremendous shearing forces which rapidly elevates the temperature of the material just prior to extrusion through the die. The duration of this is very short vs. the pre-heat time employed in a billet extrusion process, hence giving the material little time to precipitate solute. This advantage, when coupled with rod stock of the appropriate chemistry and processing history, can be used to produce certain products that have high strength through solute strengthening and/or a fine dispersion of particles. In addition the electrochemical properties of final products can be appropriately tailored for the application by introducing some alloying elements into the stock material at certain levels.

The Conform™ extrusion production process is continuous such that it greatly minimizes transverse welds, reduces possible contamination often associated with butt shearing and related pin hole leaks at billet change compared to billet extrusion, and increases recoveries. In addition, the die face pressure remains consistent, which should result in less tool wear, consistent die deflection, better dimensional tolerances, and high quality. Moreover the one-feedstock and one-extruded product process (i.e. one out process) leads to possible inline integration of other process such as flash anneal, coating, cut to length, etc.

The high strength aluminum alloys with yield strength greater than about 50 MPa that may be used in this invention would include several of the Aluminum Association's designated 1XXX, 2XXX, 3XXX, 4XXX, 5XXX, 6XXX, 7XXX and 8XXX series of aluminum alloys. Other aluminum alloys that may be used with this invention would include the alloys disclosed in U.S. Pat. Nos. 6,660,107; 6,656,296; 6,602,363; 6,503,446; 6,458,224; and 5,976,278, the contents of which are incorporated herein by reference.

This invention may also be used to produce a clad tube product by use of, but not limited to, a tangential continuous rotary extrusion process. Depending upon the final applica-

tion the clad tube can be formed with high strength aluminum alloy tube cladded with a layer of 1XXX, 2XXX, 3XXX, 4XXX, 5XXX, 6XXX, 7XXX, or 8XXX series of aluminum alloy on the exterior surface of the tube. This cladding can be subjected to a sinking or drawing ad/or an elevated thermal process (e.g. an annealing operation) to further enhance the adhesion of the cladding to the lube.

The invention also describes a method of making a heat exchanger tube that includes continuously casting a feed stock and extruding the feed stock through a continuous extrusion rotary process to form a heat exchanger tube.

In one embodiment of this method, the heat exchanger tube is quenched or air cooled after extrusion.

An aspect of this invention is to provide improved heat exchanger tubing that exhibits high strength, excellent corrosion resistance, and improved mechanical properties along with good formability, brazeability, fatigue performance and improved service life.

Another aspect of this invention is to produce micro multi void tubing exhibiting high strength, excellent corrosion resistance, and improved mechanical properties as along with good formability, brazeability and improved service life.

Another aspect of this invention is to produce small dimension tubing that exhibits high strength, excellent corrosion resistance, and improved mechanical properties with good formability, fatigue resistance, brazeability, and improved service life.

Another aspect of this invention is to produce clad tube products with high strength aluminum alloy and a clad layer or layers for corrosion resistance improvement.

Another aspect of this invention is to produce clad tube products with an outer layer of braze filler alloy such that bare fin products can be used in the manufacture of heat exchangers.

## BRIEF DESCRIPTION OF THE DRAWINGS

FIG. 1 is a cross section of a multi void heat exchanger tube;

FIG. 2 is one embodiment of a continuous rotary extrusion apparatus; and

FIG. 3 is a flowchart depicting one embodiment of the present invention.

FIG. 4 is a three-layer round tube with clad on both inside and outside of the tube.

FIG. 5 is a three-layer micro multi void tube with clad both inside and outside tube.

FIG. 6 is an enhanced round tube with a clad layer on the outside tube.

FIGS. 7a and 7b are a micro multi void tube with a clad layer.

FIG. 8 is a four-layer micro multi void tube.

## DETAILED DESCRIPTION OF PREFERRED EMBODIMENTS

The accompanying drawings and the description which follows set forth this invention in its preferred embodiments. However, it is contemplated that persons generally familiar with extrusion processes will be able to apply the novel characteristics of the structures and methods illustrated and described herein in other contexts by modification of certain details. Accordingly, the drawings and description are not to be taken as restrictive on the scope of this invention, but are to be understood as broad and general teachings. When referring to any numerical range of values, such ranges are understood to include each and every number and/or fraction between the

stated range minimum and maximum. For purposes of the description hereinafter, the terms "upper", "lower", "right", "left", "vertical", "horizontal", "top", "bottom", and derivatives thereof shall relate to the invention as it is oriented in the drawing figures.

This invention solves the difficulty of extruding a high strength alloy into a smaller, more complex structure by extruding a feedstock alloy of carefully selected chemistry and process history through a continuous rotary extrusion process. This extrusion process is known in the metal fabricating industry as the Conform™ Process, but applications of the process using high strength alloys to produce complex tubing structures is unknown. The Conform™ Process is described in U.S. Pat. No. 3,765,216, the contents of which are incorporated herein by reference. This process includes the steps of feeding metal, powder, or feedstock rod into one end of a passageway formed between first and second members, with the second member having a greater surface area for engaging the material than the first member. The passageway is blocked at one end, remote from the feeding end, and has at least one die orifice associated with the blocked end. The moving of the passageway-defining surface of the second member relative to the passage-defining surface of the first member in a direction towards the die orifice from the first end to the blocked end is such that the frictional drag of the passageway-defining surface of the second member draws the material through the passageway and generates in it a pressure that is sufficient to extrude it through the die orifice.

The advantage of using the Conform™ process to produce a small dimensional tube is three fold. First, by using the Conform™ Process a high strength feedstock alloy can be used to produce the heat exchanger tube. This advantage is possible because the feedstock in the Conform™ Process is most typically, a continuous cast rod that is smaller in diameter than a billet. The smaller diameter of the continuous cast rod significantly reduces the extrusion ratio which in turn

reduces the pressure necessary to extrude the desired product and the continuous nature of the process results in relatively constant die face pressure. Therefore, the Conform™ process allows a small size tube to be extruded using a high strength alloy. The second advantage that the Conform™ process presents is that it is cost competitive for certain difficult to extrude profiles and has the advantage of being a continuous process. The continuous process generally has high productivity and high recoveries (typically 5% process scrap or less) which in turn helps to keep the production costs competitive. Finally, by using the continuous rotary extrusion process, a non-homogenized or homogenized cast feedstock of high solute level may be used to extrude a tube that has improved strength properties and/or corrosion properties, which offers alloy design flexibility in chemistry and processing history of alloy.

It is a great advantage to achieve improved strength properties of the extruded tube by exploiting higher solute alloys, particularly continuous cast high solute alloys and having the metallurgical flexibility of using homogenized or non homogenized feedstock rod. Extruding a micro multi void tube using a non-homogenized cast billet through traditional press extrusion methods would be extremely difficult due to the high extrusion pressure that would be needed to extrude the desired product. Unlike extruding a product with a press extrusion method, the Conform™ Process requires a lower extrusion pressure since the Conform™ Process has a lower extrusion ratio. Because the Conform™ Process requires lower extrusion pressure, it is possible to extrude a small dimensional tube from a high flow stress material (e.g. a non-homogenized cast rod or high solute level alloy). By using the continuous rotary extrusion process in combination with high strength aluminum alloys and microstructures, this invention allows heat exchanger tubing to be produced with a high strength alloy while being efficient and cost competitive from a manufacturing perspective.

TABLE 1

| Metallurgical Composition of the Aluminum Alloys |                  |                  |                 |                  |                  |                                                                       |                  |                  |                  |                  |                  |                 |
|--------------------------------------------------|------------------|------------------|-----------------|------------------|------------------|-----------------------------------------------------------------------|------------------|------------------|------------------|------------------|------------------|-----------------|
| Si                                               | Cu               | Mn               | Fe              | Zn               | Ti               | Cr                                                                    | Zr               | V                | Co               | Mg               | Ni               |                 |
| about 0.01-1.5%                                  | up to about 1.2% | up to about 2.0% | about 0.01-1.0% | up to about 5.0% | up to 0.02%      | Balance substantially aluminum and incidental elements and impurities | —                | —                | —                | —                | —                | —               |
| about 0.01-1.5%                                  | up to about 1.2% | up to about 2.0% | about 0.01-1.0% | up to about 5.0% | up to 0.02%      | Balance substantially aluminum and incidental elements and impurities | about 0.01-0.35% | about 0.01-0.35% | about 0.01-0.35% | about 0.01-0.35% | up to about 1.0% | about 0.01-2.5% |
| about 0.01-1.5%                                  | up to about 1.2% | up to about 2.0% | about 0.01-1.0% | up to about 5.0% | about 0.02-0.35% | Balance substantially aluminum and incidental elements and impurities | —                | —                | —                | —                | —                | —               |

TABLE 1-continued

| <u>Metallurgical Composition of the Aluminum Alloys</u> |                  |                  |                 |                  |                   |                                                                       |                  |                  |                  |                  |                   |                 |
|---------------------------------------------------------|------------------|------------------|-----------------|------------------|-------------------|-----------------------------------------------------------------------|------------------|------------------|------------------|------------------|-------------------|-----------------|
| Si                                                      | Cu               | Mn               | Fe              | Zn               | Ti                | Cr                                                                    | Zr               | V                | Co               | Mg               | Ni                |                 |
| about 0.01-1.5%                                         | up to about 1.2% | up to about 2.0% | about 0.01-1.0% | up to about 5.0% | about 0.02-0.35%  | Balance substantially aluminum and elements and impurities            | about 0.01-0.35% | about 0.01-0.35% | about 0.01-0.35% | about 0.01-0.35% | up to about 1.0%  | about 0.01-2.5% |
| about 0.01-1.0%                                         | up to about 1.0% | up to about 1.8% | about 0.05-0.8% | up to about 2.0% | up to about 0.02% | Balance substantially aluminum and incidental elements and impurities | —                | —                | —                | —                | —                 | —               |
| about 0.01-1.0%                                         | up to about 1.0% | up to about 1.8% | about 0.05-0.8% | up to about 2.0% | up to about 0.02% | Balance substantially aluminum and incidental elements and impurities | about 0.01-0.30% | about 0.01-0.30% | about 0.01-0.30% | about 0.01-0.30% | up to about 0.08% | about 0.01-2.0% |
| about 0.01-1.0%                                         | up to about 1.0% | up to about 1.8% | about 0.05-0.8% | up to about 2.0% | about 0.02-0.30%  | Balance substantially aluminum and incidental elements and impurities | —                | —                | —                | —                | —                 | —               |
| about 0.01-1.0%                                         | up to about 1.0% | up to about 1.8% | about 0.05-0.8% | up to about 2.0% | about 0.02-0.30%  | Balance substantially aluminum and incidental elements and impurities | about 0.01-0.30% | about 0.01-0.30% | about 0.01-0.30% | about 0.01-0.30% | up to about 0.08% | about 0.01-2.0% |
| about 0.01-0.50%                                        | up to about 0.7% | up to about 1.5% | about 0.10-0.7% | up to about 1.5% | up to about 0.02% | Balance substantially aluminum and incidental elements and impurities | —                | —                | —                | —                | —                 | —               |
| about 0.01-0.50%                                        | up to about 0.7% | up to about 1.5% | about 0.10-0.7% | up to about 1.5% | up to about 0.02% | Balance substantially aluminum and incidental elements and impurities | about 0.01-0.28% | about 0.01-0.28% | about 0.01-0.28% | about 0.01-0.28% | up to about 0.08% | about 0.01-1.8% |
| about 0.01-0.50%                                        | up to about 0.7% | up to about 1.5% | about 0.10-0.7% | up to about 1.5% | about 0.02-0.25%  | Balance substantially aluminum and incidental elements and impurities | —                | —                | —                | —                | —                 | —               |
| about 0.01-0.50%                                        | up to about 0.7% | up to about 1.5% | about 0.10-0.7% | up to about 1.5% | about 0.02-0.25%  | Balance substantially aluminum and incidental elements and impurities | about 0.01-0.28% | about 0.01-0.28% | about 0.01-0.28% | about 0.01-0.28% | up to about 0.08% | about 0.01-1.8% |

## 11

Table 1 discloses the metallurgical compositions of the aluminum alloys that can be used to fabricate a heat exchanger tube in accordance with this invention. One skilled in the art would also appreciate that the heat exchanger tube can have one or more clad layers cladded over an exterior surface of the tube. The clad layer can be selected from the Aluminum Association's 1XXX, 2XXX, 3XXX, 4XXX, 5XXX, 6XXX, 7XXX, or 8XXX series of aluminum alloys.

FIG. 1 is a cross section of a multi void heat exchanger tube. FIG. 1 depicts a multi void tube 2 having a plurality of parallel flow channels 4 that are separated by a web(s) or wall(s) 6 that are aligned along the longitude of the tubing or generally perpendicular to the opposing surfaces 8 and 10. As can be seen in FIG. 1, the flow channels 4 are substantially rectangular. However, one skilled in the art would appreciate that the cross section of the flow channels 4 can have other shapes (e.g., square, circular, oval, or other regular or irregular shapes). The inner walls of the channels 4 can be smooth or rough. In making a heat exchanger, the tubes 2 are joined to corrugated fins (not shown) using a brazing process. Both multi void and micro multi void tubing 2 are about 10-25 mm in width and about 1-2 mm in height.

A high strength heat exchanger tube will soon be required as the industry adopts carbon dioxide as the standard coolant for heat exchanger systems since carbon dioxide heat exchangers operate at higher pressures than heat exchangers that utilize Freon. By using continuous casting and the Conform™ Process a heat exchanger tube can be produced with both high strength and improved corrosion resistant and service life, which will be in great favor of future automotive heat exchanger applications. A heat exchanger tube formed from a high strength and corrosion resistant aluminum alloy would not only meet the increasing demands for the new generation heat exchangers, but provide better service life and durability as well for automotives encountering salt and snow during the winter months, automobiles located in or near costal areas with high sodium chloride levels in the air, and potential corrosion from other elements or materials that might be mixed with rain water.

FIG. 2 is one example of a continuous rotary extrusion apparatus, also known as the Conform™ Process. The extrusion apparatus comprises a wheel 1 rotateably mounted on a shaft 2. The wheel 1 has a groove 3 machined around its outer edge about the axis of the wheel. A shoe member 4 fits closely against the edge of the wheel 1. An abutment member 5 formed on the underside of the shoe member 4 projects into the groove 3 and is complementary in shape to the groove cross section so as to block the groove with a sliding fit. The abutment member 5 has an extrusion orifice 6. A chamber 7 integrally formed with the shoe member 4 has a bore 8 connected with the groove 3 in the wheel 1. A sealing block 9 formed on the underside of the shoe member 4 at the opposite end to the abutment member 5 projects into and is close sliding fit in the circumferential groove 3 in the wheel 1.

The wheel 1 is rotated clockwise as shown by the arrow 11 in FIG. 2. The material 10 in the groove 3 beneath the shoe member 4 is carried forward towards the abutment member 5 by the frictional drag of the walls of the groove 3. Thus pressure is generated in the material in the groove 3, so that the material is extruded through the orifice 6 in the abutment member 5. Also the rotation of the wheel 1 drags material under a transverse shearing action from the bore 8 of the chamber 7 so that a continuous extrusion of the material is obtained.

## 12

FIG. 3 is a flowchart depicting one preferred embodiment of the inventive method. As can be understood from FIG. 3, the continuously cast feedstock rod is formed by cooling molten metal into a bar shape, which is continuously formed into a rod by a number of rollers following initial cooling. The feedstock rod is then fed into a groove located on a rotating wheel and extruded through the extrusion die to form the micro multi void tubes. After extrusion, the micro multi void tubes can then be quenched using techniques that are commonly known in the art such as water or air cooling.

FIG. 4 shows an example of a multi layer round tube 2. The multi layer tube 2 has an inner core tube 4, an intermediate layer 6, and an outer layer 8. In one application, the inner core tube 4 and the outer layer 8 are anodic (at least 20 mV more negative) to intermediate layer 6 such that the two layers enhance the corrosion resistance of the tube. However, the intermediate layer 6 can be a high strength alloy. In another application the outer layer 8 is made of a 4XXX aluminum alloy cladding for braze, the inner core tube 4 has a high magnesium content (up to 2%) for high strength, and the intermediate layer 6 has a low magnesium (up to 0.15%) content, ideally less than 0.05%, to enhance the brazeability.

FIG. 5 depicts a multi layer micro multi void tube 2. The multi layer micro multi void tube 2 has an inner core tube 4, an intermediate layer 6, and an outer layer 8. In one application the inner core tube 4 and the outer layer 8 are anodic (at least 20 mV more negative) to intermediate layer 6 such that the two layers enhance the corrosion resistance of the tube. However, the intermediate layer 6 can be a high strength alloy. In another application the outer layer 8 is made of a 4XXX series aluminum alloy cladding for braze, the inner core tube 4 has a high magnesium content (up to 2%) for high strength, and the intermediate layer 6 has a low magnesium (up to 0.15%) content, ideally less than 0.05%, to enhance the brazeability.

FIG. 6 depicts a round tube 2 with an inner core 4 and an outer layer 6. The outer layer 6 is used for applications such as braze or corrosion improvement. However, it is noted that one skilled in the art would recognize that the outer layer might be used for other applications as well yet still fall within the scope of this invention. The inner core 4 can be fabricated from a high strength alloy which can withstand high burst pressures and which exhibits enhanced heat transfer properties.

FIGS. 7a and 7b show a two layer micro multi void tube 2 having an inner core 4 and an outer layer 6. The inner core has a first end 8, a second end 10, an upper surface 12, and a lower surface 14. As depicted in FIG. 7a, the outer layer 6 can be made to cover only the upper surface 12 and the lower surface 14 of the inner core 4 while excluding the first end 8 and the second end 10. FIG. 7b depicts the outer layer 6 as covering the entire inner core 4 including the first and second ends 8 and 10.

FIG. 5 is an example of four layer micro multi void tube 2 having an inner core 4, a first intermediate layer 6, a second intermediate layer 8, and an outer layer 10. Each of the layers are designed for a specific property requirement. For example, some properties that might be desirable would include, but shall not be limited to, high strength, high corrosion resistance, solute diffusion control, and improved brazeability.

TABLE 2

| Pre and Post Braze Tensile Properties of MMV Tubing |                                |                |               |               |             |           |               |             |           |  |
|-----------------------------------------------------|--------------------------------|----------------|---------------|---------------|-------------|-----------|---------------|-------------|-----------|--|
| Alloy                                               | Feedstock                      | Homogenization | Tubing Design | Pre Braze     |             |           | Post Braze    |             |           |  |
|                                                     |                                |                |               | Tensile (MPa) | Yield (MPa) | Elong (%) | Tensile (MPa) | Yield (MPa) | Elong (%) |  |
| 1350                                                | Concast                        | No             | MMV           | 66.21         | 37.13       | 50.3      | 57.93         | 16.21       | 35.3      |  |
| High Strength Alloy (A)                             | Concast                        | No             | MMV           | 97.47         | 69.43       | 40.3      | 91.72         | 34.02       | 47.7      |  |
| High Strength Alloy (B)                             | Extruded from a DC Cast Billet | Yes            | MMV           | 91.72         | 51.95       | 43.1      | 90.00         | 30.23       | 37.4      |  |

In Table 2, the high strength alloys are the same aluminum alloy and were selected from the 3XXX series of aluminum alloys. The high strength aluminum alloy consisted essentially of about 0.01-1.0% silicon, up to about 0.70% copper, up to about 2.0% manganese; about 0.01-1.0% iron, about 0.01-5.0% zinc; about 0.01-0.35% titanium, balance substantially aluminum and incidental elements and impurities. Aluminum alloy 1350 was used as a control material.

High Strength Alloy Concast (A) and the 1350 aluminum alloy were formed into feedstock rods by a continuous casting process. The feedstock rods were then extruded into various micro multi void tubes (MMV) through the Conform™ Process. In contrast, High Strength Alloy DC Cast Billet (B) was extruded into a feedstock rod by using a traditional press extrusion method with a DC cast billet. The extruded feedstock rod was then extruded into MMV tubes through the Conform™ Process. The Conform™ Process had an extrusion ratio of 4 as compared to traditional press extrusion which has an extrusion ratio 450. Table 2 shows that when the high strength aluminum alloy is extruded through the Conform™ Process with a feedstock rod that was continuously cast and not homogenized, the extruded tube exhibited equal or higher pre and post brazed strength properties when compared to DC Cast Billet (B).

The results in Table 2 were unexpected results since one would not expect that a non-homogenized high strength alloy could be extruded to a small size MMV tube meeting all the dimensional and surface quality requirements. In addition, Table 2 shows that when the feedstock rod was formed by continuous casting (Concast (A)), the extruded MMV tube exhibited improved tensile properties over an MMV tube that was formed from a feedstock rod that was extruded from a DC cast billet using traditional press extrusion methods (DC Cast Billet (B)). For example, Table 2 shows that the Pre-braze tensile strength of the MMV tube that was formed by continuous casting (Concast (A)) had a tensile strength of 97.47 MPa, which is a 6% increase in tensile strength when compared to the MMV that was extruded DC Cast Billet (B), and a yield strength of 69.43 MPa, which is a 25% increase in yield strength when compared to the MMV that was extruded using DC Cast Billet (B). Table 2 also shows that the pre braze MMV had a 40.3% elongation. The post braze MMV that was formed by continuous casting (Concast (A)) had a tensile strength of 91.72 MPa, which is a 2% increase in tensile strength when compared to the MMV that was extruded using DC Cast Billet (B), a yield strength of 34.02 MPa, which is an 11% increase in yield strength when compared to the MMV that was extruded using DC Cast Billet (B), and an elongation of 47.7%, which is a 22% increase in elongation when compared to the MMV that was extruded using DC Cast Billet (B).

pared to the MMV that was extruded using DC Cast Billet (B). Therefore, a heat exchanger tube exhibiting improved tensile properties can be manufactured by using the Conform™ Process in combination with feedstock rod formed by continuous casting.

Since High Strength Alloy Concast (A) exhibited improved tensile properties over High Strength Alloy DC Cast Billet (B), Table 2 is an indication (for dispersion strengthened or age hardened or solute strengthened alloys) that the tensile properties of heat exchanger tubing (of like chemistry) that is extruded through a combination of continuous casting and the Conform™ Process would be greater than the tensile properties of tubing that is extruded using a billet and traditional press extrusion methods. This conclusion can be asserted because the microstructure of the extruded feedstock rod was substantially similar to that of the original billet and both the Conform™ Process and the traditional press extrusion is believed to have substantially similar metal temperatures and metal flow at the moment the metal is being extruded through the extrusion die. Therefore, it is reasonable to conclude that heat exchanger tubes extruded using the Conform™ Process would exhibit improved tensile properties over heat exchanger tubes that are extruded using a billet and traditional press extrusion methods.

TABLE 3

| Corrosion Test (SWAAT) Results (number passed over total number tested) |                         |                                    |             |         |         |         |
|-------------------------------------------------------------------------|-------------------------|------------------------------------|-------------|---------|---------|---------|
|                                                                         |                         | Rod Stock                          | Design Code | 10 Days | 20 Days | 30 Days |
| 50                                                                      | 1350                    | Concast                            | MMV         | 14/15   | 6/15    | 0/15    |
|                                                                         | High Strength Alloy (A) | Concast                            | MMV         | 15/15   | 15/15   | 15/15   |
| 55                                                                      | High Strength Alloy (B) | Extruded from a DC Cast Billet (B) | MMV         | 15/15   | 15/15   | 15/15   |
|                                                                         | High Strength Alloy (C) | Billet                             | Production  | —       | 5/5     | 5/5     |

Table 3 shows the number of extruded tubes that passed the SWAAT test in the braze condition. The SWAAT test used was the American Society for Testing and Materials (ASTM) G85 A3. The high strength alloy was selected from the 3XXX series of aluminum alloys. The high strength aluminum alloy consisted essentially of about 0.01-1.0% silicon, up to about 0.70% copper, up to about 2.0% manganese; about 0.01-1.0% iron, about 0.01-5.0% zinc; about 0.01-0.35% titanium, balance substantially aluminum and incidental elements and

15

impurities. Aluminum alloy 1350 was used as a control material and the feedstock rod was extruded using a continuous casting process.

High strength alloy continuous cast (Concast) (A), high strength alloy direct chill (DC) cast billet (B), and aluminum alloy 1350 were extruded into heat exchanger tubing using the Conform™ Process. High strength alloy billet (C) was extruded into heat exchanger tubing by using traditional press extrusion methods. Table 3 shows that the tubes extruded by the Conform™ Process with the high strength aluminum alloy exhibited similar corrosion resistance properties as compared to the tubes that were extruded with a billet by traditional press extrusion methods. As expected, the corrosion resistance of the high strength alloy was superior to that of the control 1350 aluminum alloy. Table 3 shows that the Conform™ Process can be used to produce a heat exchanger tube with identical anti-corrosive properties as that of a tube that is produced using traditional press extrusion methods.

16

0.35% titanium, and the balance substantially aluminum and incidental elements and impurities,

wherein said heat exchanger tube is formed from an aluminum alloy feedstock, said feedstock being a strip, rod, or sheet having an aspect ratio ranging from about 1:1 to 500:1, said feedstock may be exposed to elevated temperatures greater than about 300° C., said feedstock having an average secondary dendrite arm spacing less than about 100 microns and having a cross sectional area of about 2500 mm<sup>2</sup> or less and having a yield strength ranging from about 50 to about 150 MPa, and wherein said feedstock is extruded using a continuous rotary extrusion process into an extrusion.

5 15 2. The heat exchanger tube according to claim 1 wherein said extrusion is quenched or air cooled after extrusion.

10 15 3. The heat exchanger tube according to claim 1 wherein said aluminum alloy feedstock is continuously cast.

TABLE 4

| Surface Roughness Test Results of Experimental MMV Tubing |                                   |             |                     |                     |                     |                     |                     |                     |                       |
|-----------------------------------------------------------|-----------------------------------|-------------|---------------------|---------------------|---------------------|---------------------|---------------------|---------------------|-----------------------|
| Alloy-Sample ID                                           | Rod Stock                         | Design Code | R <sub>a</sub> (μm) | R <sub>q</sub> (μm) | R <sub>p</sub> (μm) | R <sub>v</sub> (μm) | R <sub>t</sub> (μm) | R <sub>z</sub> (μm) | R <sub>max</sub> (μm) |
| 1350-B23B                                                 | Concast                           | MMV         | Pass                | Pass                | Pass                | Pass                | Pass                | Pass                | Pass                  |
| High Strength Alloy                                       | Concast (A)                       | MMV         | Pass                | Pass                | Pass                | Pass                | Pass                | Pass                | Pass                  |
| High Strength Alloy                                       | Extrude from a DC Cast Billet (B) | MMV         | Pass                | Pass                | Pass                | Pass                | Pass                | Pass                | Pass                  |
| Commercially Acceptable Standards                         |                                   |             | 10                  | 10                  | 10                  | 10                  | 10                  | 10                  | 10                    |

Table 4 shows the pre braze surface roughness measurements of the tubes that were extruded using the Conform™ Process. As with the previous trials, the high strength alloy was selected from the 3XXX series of aluminum alloys. Aluminum alloy 1350 was used as a control material. All of the alloys were extruded into a micro multi void (MMV) tube. The measurements were taken normal to the extrusion direction and the measurements include the following: R<sub>a</sub>—roughness average, R<sub>q</sub>—root mean squared roughness average, R<sub>p</sub>—maximum peak height, R<sub>v</sub>—maximum valley depth, R<sub>t</sub>—maximum roughness depth, R<sub>z</sub>—mean peak-to-valley height, and R<sub>max</sub>—Maximum peak-to-valley height.

Table 4 shows that the tubes that were extruded using the Conform™ Process exceed the current commercially acceptable standards in the relevant industry. This result was the same regardless if the feedstock rod was formed by continuous casting or by extrusion by a DC cast billet. Therefore, a heat exchanger tube with small dimensions and improved tensile properties can be produced using the Conform™ Process with surface roughness equivalent to that of tubes extruded using traditional press extrusion methods.

Having described the presently preferred embodiments, it is to be understood that the invention may be otherwise embodied within the scope of the appended claims.

What is claimed is:

1. A heat exchanger tube having improved resistance to high burst pressures, said heat exchanger tube comprising an aluminum alloy that consists essentially of about 0.01-1.5% silicon, tip to about 1.2% copper, tip to about 2.0% manganese, about 0.01-1.0% iron, up to about 5.0% zinc, tip to about

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 933

**17**

13. The heat exchanger tube according to claim 1 wherein said tube has an electric conductivity that is above about 48% IACS.

14. The heat exchanger tube according to claim 1 wherein said tube has a post-braze electric conductivity that is above about 48% IACS.

15. The heat exchanger tube according to claim 1 wherein the titanium ranges about 0.02% to about 0.35% titanium.

16. The heat exchanger tube according to claim 1 wherein said aluminum alloy further contains one or more of the following elements: up to about 0.8% magnesium, about 0.01-0.30% chromium, about 0.01-0.30% zirconium, about 0.01-0.30% vanadium, about 0.01-0.30% cobalt, and about 0.01-2.0% nickel.

17. The heat exchanger tube according to claim 1 wherein said aluminum alloy further contains one or more of the following elements: up to about 0.8% magnesium, about 0.01-0.28% chromium, about 0.01-0.28% zirconium, about 0.01-0.28% vanadium, about 0.01-0.28% cobalt, and about 0.01-1.8% nickel.

18. The multi layered extruded tube according to claim 1, further comprising one or more clad layers comprising an aluminum alloy selected from the group consisting essentially of the 1XXX, 2XXX, 3XXX, 4XXX, 5XXX, 6XXX,

**18**

7XXX, and 8XXX series of aluminum alloys cladded on an exterior surface of said inner core.

19. The multi layered extruded tube according to claim 18 wherein an exterior surface of said extrusion is cladded with one or more clad layers by using one or more tangential continuous rotary extrusion machines.

20. The multi layered extruded tube according to claim 18 wherein said clad layers are drawn or sanked over said inner core tube after cladding.

21. The multi layered extruded tube according to claim 18 wherein said clad layer is selected from the group consisting essentially of aluminum alloys 4343, 4045, and 4047, said clad layer having a thickness ranging from about 3  $\mu\text{m}$  to about 300  $\mu\text{m}$ .

22. The multi layered extruded tube according to claim 18 wherein one clad layer has an electrochemical potential difference of at least about 20 mV to about 40 mM when compared to said inner core tube or an adjacent clad layer.

23. The multi layered extruded tube according to claim 18, wherein one or more tangential continuous rotary extrusion machines are used to clad one or more clad layers onto said exterior surface of said inner core tube.

\* \* \* \* \*

UNITED STATES PATENT AND TRADEMARK OFFICE  
**CERTIFICATE OF CORRECTION**

PATENT NO. : 7,732,059 B2

Page 1 of 1

APPLICATION NO. : 11/157668

DATED : June 8, 2010

INVENTOR(S) : Baolute Ren, Raymond J. Kilmer and John F. Butler, Jr.

It is certified that error appears in the above-identified patent and that said Letters Patent is hereby corrected as shown below:

In claim 1, column 15, line 63, after “exchanger”, delete “tithe” and insert -- tube --.

In claim 1, column 15, line 66, after “silicon,”, delete “tip” and insert -- up --.

In claim 1, column 15, line 66, after “copper,”, delete “tip” and insert -- up --.

In column 15, line 67, after “zinc,”, delete “tip” and insert -- up --.

In column 17, line 17, after “elements:”, delete “tip” and insert -- up --.

In column 18, line 12, after “consisting”, delete “essentially”.

Signed and Sealed this

Fifth Day of October, 2010



David J. Kappos  
Director of the United States Patent and Trademark Office